

# United States Patent Office

3,077,370

Patented Feb. 12, 1963

1

3,077,370

## DYEING OF CELLULOUS MATERIAL WITH VAT DYESTUFFS

William Kilby and Cedric Hitchen, Lancaster, England, assignors to Standfast Dyers & Printers Limited, Lancaster, England, a British company  
No Drawing. Filed Mar. 26, 1959, Ser. No. 892,044  
Claims priority, application Great Britain Apr. 8, 1958  
5 Claims. (Cl. 8—34)

This invention relates to a process for dyeing cellulosic material with vat dyestuffs.

A previously proposed process for the continuous dyeing of cellulosic materials with vat dyestuffs comprises impregnating the material with a fine aqueous suspension of the dyestuff, removing the surplus liquor by passing the material through a padding mangle, treating the material with an alkaline reducing solution (usually an aqueous solution of caustic soda and sodium hydrosulphite), and passing the material through a bath of molten metal. The soluble alkaline leuco-compound of the vat dyestuff, formed by the alkaline reducing solution, has an affinity for the cellulosic material, and the dyestuff is therefore fixed in the material. However, due to the speed of this continuous process, full reduction and fixation of the dyestuff is not always obtained. Also, any attempt to ensure full reduction and fixation by applying to the material in some degree at the padding stage an alkaline solution of leuco compounds instead of an aqueous suspension of dyestuff, results in "tailing" difficulties due to the affinity of the leuco compounds for the cellulosic material.

It has also previously been proposed to dye cellulosic material with vat dyestuff by impregnating the material with a suspension of acid leuco vat dyestuff prepared by reducing the vat dyestuff with thiourea dioxide at an elevated temperature under neutral or acid conditions, allowing such acid leuco vat dyestuff to oxidize to vat dyestuff in finely divided form within the cellulosic material, and thereafter subjecting the material to alkaline reduction to fix the vat dyestuff upon the fibre. In this case, the acid leuco vat dyestuff has little affinity for cellulosic material and "tailing" is therefore avoided. However, the process is slowed somewhat by the step of oxidizing the acid leuco vat dyestuff, and moreover the process involves transfer of the material to a jigger in which the alkaline reduction step is effected.

An object of the invention is to provide a speedy, economical and continuous vat dyeing process in which "tailing" difficulties are avoided.

According to the invention a process of dyeing cellulosic material with vat dyestuff comprises impregnating the material with a suspension of acid leuco vat dyestuff and while the dyestuff in the material is in the acid leuco form treating the material with an alkaline liquor so as to convert the dyestuff in the material to the alkaline leuco form.

Thus, the alkaline leuco compound of the dyestuff is formed directly within the material, the steps of the oxidation of the acid leuco compound and treatment with the usual reducing chemicals being avoided. Also, there are no "tailing" difficulties at the padding mangle.

Preferably the material with alkaline leuco dyestuff therein is passed through a heater to complete the fixation of the dyestuff.

Preferably also the heater consists of a molten metal continuous dyeing machine. In this connection, it is found that suspensions of the acid leuco-compounds of vat dyestuffs, when prepared by the neutralisation with acid, in the presence of a suitable dispersing agent, of the alkaline leuco-compounds, contain decomposition products of the sodium hydrosulphite used for reduction.

2

Such decomposition products, particularly the sulphides formed, attack the molten metal of the continuous dyeing machine, causing formation of a sulphide scum and excessive loss of metal.

5 This disadvantage is avoided according to a further feature of the invention by use of a suspension of acid leuco vat dyestuff produced by treating the vat dyestuff with thiourea dioxide at elevated temperature and under neutral or acid conditions.

10 Preferably also the alkaline treating liquor floats on the surface of the molten metal at the entry to the molten metal.

The alkaline treating liquor may be an aqueous solution of caustic soda, or of caustic soda containing sodium 15 hydrosulphite.

Materials dyed by the process according to the invention are of good appearance, well-penetrated and in the case of most dyestuffs, fuller in shade than comparable dyeings produced by the application of the vat dyestuffs themselves at the padding stage.

20 The following examples are given, but merely to illustrate the invention:

### Example 1

25 A liquor containing the following quantities of vat dyestuff and chemicals was heated to 90–95° C. for five minutes with constant stirring:

|                                                     | Gms./litre |
|-----------------------------------------------------|------------|
| Caledon Golden Orange 3G single paste (I.C.I.)      |            |
| 30 (Colour Index Vat Orange 15) -----               | 100        |
| Dispersol AC (I.C.I.) (the disodium salt of methyl- |            |
| ene dinaphthalene sulphonic acid) -----             | 5          |
| Caledon Salt A (I.C.I.) (the sodium salt of anthra- |            |
| 35 quinone-2-sulphonic acid) -----                  | 1          |
| Disodium hydrogen orthophosphate -----              | 5          |
| Thiourea dioxide -----                              | 20         |

20 A fine suspension of the acid leuco-compound of Caledon Golden Orange 3G was produced.

40 This suspension of the acid leuco-compound of the dyestuff was cooled to 60° C. and cotton cloth was impregnated evenly with the suspension on a padding mangle, in such a way that the material retained about 70% of its own weight of padding liquor. Directly after impregnation, the material was passed through a molten metal continuous dyeing machine as described in our British patent specification No. 620,584. The molten metal was maintained at a temperature of 95° C. and the floating bath at the entry to the molten metal contained an aqueous solution of caustic soda, 40 gms./litre, and sodium hydrosulphite 5 gms./litre, at 90° C. The dyeing was then completed in the ordinary way by oxidation, soaping and rinsing.

50 The orange dyeing produced was of excellent appearance, penetration and levelness.

### Example 2

60 A liquor containing the following amounts of vat dyestuff and chemicals was heated to the boil for 5 minutes and then allowed to cool to 60° C.:

|                                                    | Gms./litre |
|----------------------------------------------------|------------|
| Caledon Blue XRC single paste (Colour Index Vat    |            |
| 65 Blue 6) (trichloro-n-dihydro - 1:2:1:2'-anthra- |            |
| quinoneazine) -----                                | 250        |
| Dispersol AC -----                                 | 5          |
| Caledon Salt A -----                               | 1          |
| Disodium hydrogen orthophosphate -----             | 5          |
| Thiourea dioxide -----                             | 50         |

70 Cotton fabric was impregnated evenly, at the padding mangle, with the suspension of the acid leuco-compound of Caledon Blue XRC thus obtained, the padded ma-

terial retaining approximately 70% of its own weight of the padding liquor.

Directly after padding, the fabric was passed through the molten metal dyeing machine of Example 1, the molten metal being maintained at 95° C. The floating entry bath of the machine contained an aqueous solution of caustic soda of 40 gms./litre at 90° C. The dyeing was completed in the normal manner by oxidation, soaping and washing.

*Example 3*

A liquor containing the following amounts of vat dyestuff and chemicals was heated to 90-95° C. for 5 minutes with constant stirring:

|                                                                          | Gms./litre | 15 |
|--------------------------------------------------------------------------|------------|----|
| F.D. Caledon Brilliant Orange 6R powder fine (Colour Index Vat Orange 3) | 30         |    |
| Dispersol AC                                                             | 5          |    |
| Caledon Salt A                                                           | 1          |    |
| Disodium hydrogen orthophosphate                                         | 5          | 20 |
| Thiourea dioxide                                                         | 50         |    |

The suspension of the acid leuco-compound of the dyestuff so formed was cooled to 60° C. and applied evenly to cotton fabric by padding, the material retaining approximately 70% of its own weight of the padding liquor.

Directly after padding, the material was continuously passed through the molten metal dyeing machine of Example 1, the molten metal being maintained at 95° C. The entry bath of the machine contained an aqueous solution of caustic soda of 40 gms./litre at 90° C., and the dyeing was completed in the normal manner by oxidation, soaping and washing.

The resultant dyeing was of excellent appearance, penetration and levelness and deeper in shade than a comparable dyeing produced by the normal process in which a suspension of the unreduced vat dyestuff was applied at the padding stage.

*Example 4*

A liquor containing the following amounts of chemicals and vat dyestuffs was heated to 90-95° C. for 5 minutes with constant stirring:

|                                                                                                                                                                                                                                                                                                                     | Gms./litre | 45 |
|---------------------------------------------------------------------------------------------------------------------------------------------------------------------------------------------------------------------------------------------------------------------------------------------------------------------|------------|----|
| Caledon Brown R single paste (Colour Index Vat Brown 3) (the dyestuff obtained by treating 4:5-dibenzoylaminio-1:1'-dianthrimide with sulphuric acid, c.f. Thorpe's Dictionary of Applied Chemistry, fourth edition, vol. I, p. 422)                                                                                | 45         | 50 |
| Caledon Brown G single paste (Colour Index Vat Brown 3 mixed with Colour Index Vat Black 27) (a mixture of the dyestuff obtained by treating 4:4'-dibenzoylaminio-1:1'-dianthrimide with sulphuric acid, c.f. Thorpe's Dictionary of Applied Chemistry, fourth edition, vol. I, p. 422, and Caledon Brown RS above) | 32         | 50 |
| Caledon Dark Brown 3R single paste (Colour Index Vat Brown 1)                                                                                                                                                                                                                                                       | 11.5       | 55 |
| Dispersol AC                                                                                                                                                                                                                                                                                                        | 5          |    |
| Caledon Salt A                                                                                                                                                                                                                                                                                                      | 1          |    |
| Disodium hydrogen orthophosphate                                                                                                                                                                                                                                                                                    | 5          | 25 |
| Thiourea dioxide                                                                                                                                                                                                                                                                                                    | 25         |    |

The resultant fine suspension of the acid leuco-compounds of the dyestuffs was allowed to cool to 60° C. and then applied evenly to linen fabric by a padding process. Directly after padding, the fabric was passed through the molten metal dyeing machine of Example 1, the molten metal being maintained at 95° C. The entry bath of the machine contained an aqueous solution of caustic soda, 40 gms./litre and sodium hydrosulphite 5 gms./litre at 90° C. Dyeing was completed in the normal way by oxidation, soaping and washing.

The tan shade produced was of excellent appearance, levelness and penetration.

The invention also comprises cellulosic materials whenever dyed with vat dyestuffs by any of the foregoing processes according to the invention.

Use may also be made of the inventions described in our British patent specifications Nos. 661,086, 663,066, 665,454 and 681,983.

We claim:

1. A process of dyeing cellulose with vat dyestuff, comprising impregnating a continuous length of cellulose with a suspension of a thiourea dioxide-reduced acid leuco vat dyestuff, treating the impregnated cellulose with an alkaline liquor, while the dyestuff in the material is in the acid leuco form, so as to convert the dyestuff to the alkaline leuco form, and passing the cellulose through the molten metal of a molten metal continuous dyeing machine to complete the fixation of the dyestuff.
2. A process according to claim 1, wherein the molten metal is maintained at approximately 95° C.
3. A process according to claim 2, wherein the alkaline treating liquor is a hot aqueous liquor floating on the surface of the molten metal at the entry to the molten metal.
4. A process according to claim 3, wherein the alkaline treating liquor is a hot aqueous solution of caustic soda.
5. A process according to claim 3, wherein the alkaline treating liquor is a hot aqueous solution of caustic soda and sodium hydrosulphite.

References Cited in the file of this patent

UNITED STATES PATENTS

|           |               |                |
|-----------|---------------|----------------|
| 2,256,808 | Kern          | Sept. 23, 1941 |
| 2,447,993 | Vieira        | Aug. 24, 1948  |
| 2,487,197 | Stott et al.  | Nov. 8, 1949   |
| 2,693,995 | Hannay et al. | Nov. 9, 1954   |

FOREIGN PATENTS

|    |         |               |               |
|----|---------|---------------|---------------|
| 50 | 620,584 | Great Britain | Mar. 28, 1949 |
|    | 702,040 | Great Britain | Jan. 6, 1954  |
|    | 702,050 | Great Britain | Jan. 6, 1954  |
|    | 765,335 | Great Britain | Jan. 9, 1957  |